

## UNITED STATES PATENT OFFICE

2,627,507

## PAD DYEING COMPOSITION

Joseph M. Kuhn, Haddonfield, N. J., assignor to  
The Sherwin-Williams Company, Cleveland,  
Ohio, a corporation of Ohio

No Drawing. Application July 20, 1951,  
Serial No. 237,833

15 Claims. (Cl. 260—15)

1

This invention relates, as indicated, to an improved pad dyeing composition. More particularly, this invention relates to compositions which are particularly adaptable to pad dyeing for textiles having discrete fibers with insoluble pigments to produce a solid colored textile. In pad dyeing there is usually employed a bath comprising an emulsion of water and a volatile solvent, the latter containing the pigment and the resin binder or binders. One method of pad dyeing is to immerse the textile in the bath and then pass it between squeeze rolls which remove the excess of color and other bath constituents. As an alternate method, one of the squeeze rolls may be partially immersed in the color bath, whereby some of the bath is carried to the nip between the partially immersed roll and the roll adjacent to it. In this case the textile is dyed by passing between the rolls without previous immersion in the bath. A method of pad dyeing resin-bound water-insoluble pigments in a water emulsion has been disclosed by Jennings in Patent 2,344,199.

Although pigmented lacquer-in-water emulsions have been known and recommended for dyeing textiles, a serious drawback has been the difficulty of preparing emulsions which will remain stable over a long period of time, and under those conditions which exist in the pad dyeing process where the textile and the emulsion are continuously squeezed between two or more tightly set squeeze rolls, this condition is more pronounced. Previous technique in the preparation of such textile coating compositions has specified the use of a volatile solvent for the resinous binder, which solvent has been either a water-soluble organic solvent or a water-insoluble organic solvent. The compositions of this invention are not properly designated as "lacquer-in-water" emulsion since there is no substantial amount of solvent for the resin present therein. Water is, however, the external phase, and resin, plasticizer and pigment (which is dispersed in the resin) constitutes the internal or discontinuous phase. For all practical purposes, these compositions are solvent-free as will be more clearly explained hereinafter and will be designated as "resin-in-water" emulsions.

It is a novel feature of my invention to provide pad dyeing compositions and a method of em-

2

ploying the same which compositions contain no volatile water-insoluble organic solvents for the resin, such as commonly employed heretofore, and relatively minor proportions, on the order of less than 1%, of volatile water-soluble organic solvents for the resin. In addition to the ordinary advantages obtained in eliminating a solvent from any system, namely, economy and avoidance of the usual hazards encountered when employing solvents, it has been found most unexpectedly that extremely fine dispersions are obtainable resulting in a uniform dyeing effect when the material is padded, dried, and cured and improved fastness properties are obtained. For the purposes of this invention and the ensuing disclosure, "volatile solvents" are to be considered volatile when the boiling point at atmospheric pressure is less than 225° C.

The compositions of this invention differ materially from those heretofore employed in that no reliance is made upon the presence of volatile solvents to secure adequate penetration and even dyeing.

It is, therefore, a principal object of this invention to provide a substantially volatile solvent-free pad dyeing composition.

Other objects of this invention will appear as the description proceeds.

To the accomplishment of the foregoing and related ends, said invention, then, consists of the means hereinafter fully described and particularly pointed out in the appended claims, the following description setting forth in detail certain illustrative embodiments of the invention, such disclosed means constituting, however, but a few of the various forms in which the principle of this invention may be employed.

Broadly stated, therefore, this invention comprises the provision of a resin-water emulsion suitable for use in pad dyeing baths in which the resinous binder comprises a water-insoluble cellulose ether, a water-insoluble alkylated melamine-aldehyde resin and a non-volatile plasticizer, said resinous binder having dispersed therein a water-insoluble pigment, and in which emulsion the aqueous phase comprises water, said emulsion being free of water-insoluble organic solvents and containing less than 5% by weight of a water-soluble organic solvent. Film-forming ingredients are to be considered, for the pur-

poses of this invention, as including the melamine-aldehyde resin, the cellulose ether, the plasticizer and other such organic materials which remain on drying in the film. The term is exclusive of pigments and the aqueous phase.

The compositions of this invention are usually prepared in the form of a concentrate which is diluted with water by the ultimate user to a proper consistency and depth of color for pad dyeing. Examples which are given below, provide concentrates. These concentrates are employed in amounts ranging from 0.05% to about 5%, water constituting the balance, to provide a suitable pad dyeing bath. When so diluted, the compositions of this invention as padded will contain from about 0.01% to no more than 1% by weight of a volatile water-soluble organic solvent. Most generally, the amount of such solvent in the dye bath is no more than 0.25% by weight.

In the concentrated form, the amount of such solvent will be proportionately larger ranging from 0.05 to about 5%, more generally, 2.5% or less. The only reason any volatile water-soluble organic solvent is present at all in any of these compositions is to facilitate handling of the melamine-aldehyde resin in compounding operations. Such solvent serves no other useful purpose and is, therefore, unnecessary in the final compositions.

The alkylated melamine formaldehyde condensation products which are useful in accordance with this invention may be prepared by known methods. For example, reference may be had to the patent to Widmer, 2,197,357, and the patent to Swain, Re. 22,402. In general, these condensation products are prepared by reacting 2 to 6 mols of formaldehyde with 1 mol of melamine. The condensation product formed is believed to be mostly methylol-melamine.

When preparing the various alkylated melamine formaldehyde condensation products, it is frequently desirable to prepare first the methylated methylol-melamine and then, by an interchange process utilizing an aliphatic alcohol of the desired carbon atom content, e. g., 3 to 12 carbon atoms, obtain the corresponding "alkylated" methylol-melamine. Specific examples of such treatment are also given in the patent to Johnstone et al., Re. 22,566.

Specific examples of the alkylated melamine formaldehyde condensation products which may be used in accordance with this invention include propylated methylol-melamine, butylated methylol-melamine, hexylated methylol-melamine, cyclohexylated methylol-melamine, caprylated methylol-melamine, laurylated methylol-melamine, etc.

A preferred material for use in accordance with this invention is the butylated melamine-formaldehyde product, primarily because of its ready availability on the market, and for this reason it has been used in the specific examples which follow at a later point in the specification, but which will be understood as merely illustrative of the use of other such alkylated methylol-melamines. The melamine-aldehyde resins containing less than 3 carbon atoms in the alkyl group tend to be too soluble in water for the purposes of this invention.

The water-insoluble cellulose ethers which have been found to be useful in accordance with this invention include aliphatic cellulose ethers, e. g., ethyl cellulose, propyl cellulose, butyl cellulose, benzyl cellulose, mixed ethyl benzyl cellulose, mixed ethyl butyl cellulose, etc. In general,

these ethers are sufficiently etherified to be insoluble in water. For example, ethyl cellulose, which is preferred, will have an ethoxy content within the range of from about 40% to about 50%, and preferably from about 47% to about 48.5%. Such a material is available on the market and has a viscosity of 10 centipoises. The alkyl cellulose ethers are a preferred class.

In general, the amount of melamine-formaldehyde resin is in excess of the amount of cellulose ether. It has been found that wash fastness is impaired if there be more than 1 part of cellulose ether to 1 part of resin by weight.

The emulsion as marketed may have a non-aqueous phase greater than 50%, but when used for pad dyeing, it is greatly diluted with water.

It becomes convenient at this point to illustrate the manner of compounding the compositions of this invention by giving several specific examples which are to be understood as being illustrative of the principles of this invention and not for the purpose of limiting the invention to the precise compositions which are shown.

#### EXAMPLE I

1000 grams of Melmac 245-8 (a butylated melamine formaldehyde resin composition containing 50% butylated melamine formaldehyde, 30% butyl alcohol and 20% xylol) and 500 grams of dibutyl phthalate were mixed together and passed over a three roll mill several times until the volatile solvent was completely evaporated. Using this resin-plasticizer mixture, a padding color was made as follows:

1085 grams of monastral blue presscake (copper phthalocyanine) containing 200 grams of pigment, and 100 grams of a 50% aqueous solution of a sodium salt of a naphthalene sulphonic acid-formaldehyde condensation product (Blancol) were mixed to yield a dispersion. To this mixture were then added 100 grams of butyl Cellosolve and 300 grams of the above resin-plasticizer mixture. The pigment was then flushed into the lacquer phase from the aqueous phase and 970 grams of water, butyl Cellosolve and a dispersing agent were removed. The resulting composition was then washed three successive times with 800 gram portions of water following which there were removed 806 grams of water and butyl Cellosolve, 803 grams of water and butyl Cellosolve and 826 grams of water and butyl Cellosolve, respectively. 200 grams of ethyl cellulose (10 centipoise standard ethoxy) were then added and the batch mixed to dissolve. An additional 500 grams of the above resin plasticized mixture were then added together with 104 grams of oleic acid, 52 grams of triethanolamine, 1500 grams of water and 15 grams of ammonia (27% NH<sub>3</sub>).

The pigmented resin plasticizer mixture was very well dispersed in water and found to remain stable on storage for periods of up to 2 to 3 years. This printing paste contains no water-insoluble volatile organic solvents, the only volatile solvent employed being butyl Cellosolve which is completely soluble in water. The repeated washings with water effectively removed from the composition all but a very minor percentage of such solvent.

Dyeings made with the above color composition according to the usual pad dyeing technique showed excellent appearance and fastness properties.

Amylated melamine-formaldehyde resin may be used in place of part or all of the butylated melamine-formaldehyde resin of this example.

## EXAMPLE II

In this example there was used a solvent-free solid form of butylated melamine-formaldehyde resin known as Resimene 888. The materials employed, with brief indications as to the steps, are as follows:

|                                                                 |    |
|-----------------------------------------------------------------|----|
| 1,466 gm. Monastral Blue press cake (300 gm. pigment)           | 5  |
| 150 gm. Blancol solution 50%                                    | 10 |
| Mix to disperse                                                 |    |
| 150 gm. butyl Cellosolve                                        |    |
| 240 gm. Resimene 888                                            |    |
| 240 gm. dibutyl phthalate                                       |    |
| Flush and remove 1,273 gms. water and 15 butyl Cellosolve. Add: | 15 |
| 500 gm. water                                                   |    |
| Wash and remove 534 gm. water                                   |    |
| 150 gm. ethyl cellulose (10 cp. standard ethoxy)                | 20 |
| Mix until dissolved                                             |    |
| 166 gm. oleic acid                                              |    |
| 83 gm. monoethanolamine                                         |    |
| 1,425 gm. water                                                 |    |
| 37 gm. ammonia (27% NH <sub>3</sub> )                           | 25 |
|                                                                 |    |
| 4,607 gm.                                                       |    |

Butyl Cellosolve is a monobutyl ether of ethylene glycol. Other pigments may, of course, be employed.

## EXAMPLE III

The materials employed, with a brief indication as to the steps, are as follows:

|                                                      |    |
|------------------------------------------------------|----|
| 941 gm. Monastral Green press cake (250 gm. pigment) | 35 |
| 41 gm. Blancol solution 50%                          |    |
| 100 gm. butyl Cellosolve                             |    |
| 200 gm. Resimene 888                                 |    |
| 200 gm. dibutyl phthalate                            | 40 |
| Flush and remove 652 gm. water. Add:                 |    |
| 500 gm. water                                        |    |
| Wash and remove 534 gm. water                        |    |
| 125 gm. ethyl cellulose (10 cp. standard ethoxy)     | 45 |
| Mix to dissolve                                      |    |
| 138 gm. oleic acid.                                  |    |
| 69 gm. triethanolamine                               |    |
| 1,257 gm. water                                      |    |
| 30 gm. ammonia (27% NH <sub>3</sub> )                |    |
|                                                      |    |
| 3,601 gm.                                            |    |

## EXAMPLE IV

The materials employed, with a brief indication as to the steps, are as follows:

|                                                        |    |
|--------------------------------------------------------|----|
| 1,129 gm. Monastral Green press cake (300 gm. pigment) | 55 |
| 49 gm. Blancol solution 50%                            | 60 |
| Mix to disperse                                        |    |
| 100 gm. butyl Cellosolve                               |    |
| 240 gm. Resimene 888                                   |    |
| 240 gm. dibutyl phthalate                              |    |
| Flush and remove 773 gm. water                         | 65 |
| 500 gm. water                                          |    |
| Wash and remove 513 gm. water                          |    |
| 150 gm. ethyl cellulose (10 cp. standard ethoxy)       |    |
| Mix until dissolved                                    |    |
| 80 gm. oleic acid                                      |    |
| 40 gm. triethanolamine                                 |    |
| 861 gm. water                                          |    |
| 37 gm. ammonia (27% NH <sub>3</sub> )                  |    |
|                                                        |    |
| 3,426 gm.                                              |    |

## EXAMPLE V

The materials employed, with a brief indication as to the steps, are as follows:

## Resin solution

|                          |                                |
|--------------------------|--------------------------------|
| 500 gm. Resimene 888     | Mix thoroughly until dissolved |
| 250 gm. butyl Cellosolve |                                |
| 250 gm. butyl cellosolve |                                |

1,000 gm.

## Padding color

|                                                     |    |
|-----------------------------------------------------|----|
| 454 gm. Monastral Blue press cake (136 gm. pigment) | 25 |
| 68 gm. Blancol solution 50%                         |    |
| 217 gm. above resin solution                        |    |
| Flush and remove 358 gm. water                      |    |
| 68 gm. ethyl cellulose (10 cp. standard ethoxy)     | 30 |
| Mix until dissolved. Add:                           |    |
| 300 gm. water                                       |    |
| Wash and remove 253 gm. water. Add:                 |    |
| 300 gm. water                                       |    |
| Wash and remove 286 gm. water. Add:                 |    |
| 300 gm. water                                       |    |
| Wash and remove 305 gm. water                       |    |
| 50 gm. Pflaumer's ester P-153-S                     |    |
| 50 gm. Triton X-100                                 |    |
| 20 gm. ammonia (27% NH <sub>3</sub> )               |    |
| 375 gm. water                                       |    |

2,202 gm.

Ester P-153-S, is a fatty acid ester of a mannitol or sorbitol type alcohol. Triton X-100 is an ethylene oxide condensation product. Both are emulsifiers.

All the ethyl cellulose used in the following experiments is of the 10 cp., 46.8-48.5% ethoxy content type.

The following example employs the resin, ethyl cellulose, plasticizer, and water soluble solvents in a single solution.

## EXAMPLE VI

The materials employed, with a brief indication as to the steps, are as follows:

|                                                |    |
|------------------------------------------------|----|
| 50 gm. Monastral Blue press cake (272 pigment) | 50 |
| 136 gm. Blancol solution 50%                   |    |
| Mix together to disperse                       |    |
| 217 gm. Resimene 888                           |    |
| 209 gm. butyl Cellosolve                       |    |
| 108 gm. dibutyl phthalate                      | 55 |
| Premix and dissolve                            |    |
| 136 gm. ethyl cellulose                        |    |
| Flush and remove 500 gm. water                 |    |
| 600 gm. water                                  | 60 |
| Wash and remove 620 gm. water                  |    |
| 600 gm. water                                  |    |
| Wash and remove 655 gm. water                  |    |
| 690 gm. water                                  |    |
| Wash and remove 630 gm. water                  |    |
| 100 gm. Pflaumer's ester P-153-S               | 65 |
| 100 gm. Triton X-100                           |    |
| 40 gm. ammonia (27% NH <sub>3</sub> )          |    |
| 1,081 gm. water                                |    |

## EXAMPLE VII

The materials employed, with a brief indication as to the steps, are as follows:

|                                                      |                     |
|------------------------------------------------------|---------------------|
| 464 gm. Monastral Green press cake (140 gm. pigment) | Premix and dissolve |
| 109 gm. Resimene 888                                 |                     |
| 54 gm. dibutyl phthalate                             | 5                   |
| 54 gm. ethyl alcohol                                 |                     |
| Flush and remove 313 gm. water                       | 10                  |
| 68 gm. ethyl cellulose                               |                     |
| 50 gm. ethyl alcohol                                 | 15                  |
| Mix until dissolved                                  |                     |
| 300 gm. water                                        | 20                  |
| Wash and remove 300 gm. water                        |                     |
| 300 gm. water                                        | 25                  |
| Wash and remove 300 gm. water                        |                     |
| 50 gm. Pflaumer's ester P-153-S                      | 30                  |
| 50 gm. Triton X-100                                  |                     |
| 25 gm. ammonia (27% NH <sub>3</sub> )                | 35                  |
| 389 gm. water                                        |                     |
| 1,913 gm.                                            |                     |

## EXAMPLE VIII

The materials employed, with a brief indication as to the steps, are as follows:

|                                                     |    |
|-----------------------------------------------------|----|
| 464 gm. Monastral Blue press cake (140 gm. pigment) | 25 |
| 109 gm. Resimene 888                                |    |
| 54 gm. dibutyl phthalate                            | 30 |
| 54 gm. acetone                                      |    |
| Flush and remove 319 gm. water                      | 35 |
| 68 gm. ethyl cellulose 10 cp.                       |    |
| Mix to dissolve                                     | 40 |
| 300 gm. water                                       |    |
| Wash and remove 300 gm. water                       | 45 |
| 50 gm. Pflaumer's ester P-153-S                     |    |
| 50 gm. Triton X-100                                 | 50 |
| 25 gm. ammonia (27% NH <sub>3</sub> )               |    |
| 445 gm. water                                       |    |
| 1,619 gm.                                           |    |

This example starts with a pigment pres cake instead of a water dispersion, and uses a water-soluble volatile organic solvent other than butyl Cellosolve.

## EXAMPLE IX

The materials employed, with a brief indication as to the steps, are as follows:

|                                                      |    |
|------------------------------------------------------|----|
| 464 gm. Monastral Green press cake (140 gm. pigment) | 50 |
| 109 gm. Resimene 888                                 |    |
| 54 gm. dibutyl phthalate                             | 55 |
| 54 gm. methyl Cellosolve                             |    |
| Flush and remove 331 gm. water                       | 60 |
| 68 gm. ethyl cellulose 10 cp.                        |    |
| Mix and dissolve                                     | 65 |
| 300 gm. water                                        |    |
| Wash and remove 300 gm. water                        | 70 |
| 300 gm. water                                        |    |
| Wash and remove 300 gm. water                        | 75 |
| 50 gm. Pflaumer's ester P-153-S                      |    |
| 50 gm. Triton X-100                                  | 80 |
| 25 gm. ammonia (27% NH <sub>3</sub> )                |    |
| 457 gm. water                                        |    |
| 1,931 gm.                                            |    |

This example uses still another water soluble volatile organic solvent.

## EXAMPLE X

The materials employed, with a brief indication as to the steps, are as follows:

|                                                      |    |
|------------------------------------------------------|----|
| 464 gm. Monastral Green press cake (140 gm. pigment) | 8  |
| 109 gm. Resimene 888                                 |    |
| 54 gm. tetrahydroabietyl alcohol                     | 10 |
| 54 gm. butyl Cellosolve                              |    |
| Flush and remove 261 gm. water                       | 15 |
| 68 gm. ethyl cellulose 10 cp.                        |    |
| 16 gm. butyl Cellosolve                              | 20 |
| Mix to dissolve                                      |    |
| 300 gm. water                                        | 25 |
| Wash and remove 307 gm. water                        |    |
| 300 gm. water                                        | 30 |
| Wash and remove 300 gm. water                        |    |
| 300 gm. water                                        | 35 |
| Wash and remove 301 gm. water                        |    |
| 50 gm. Pflaumer's ester P-153-S                      | 40 |
| 50 gm. Triton X-100                                  |    |
| 25 gm. ammonia (27% NH <sub>3</sub> )                | 45 |
| 379 gm. water                                        |    |
| 2,169 gm.                                            |    |

Uses an alcohol-type plasticizer.

## EXAMPLE XI

The materials employed, with a brief indication as to the steps, are as follows:

|                                                      |    |
|------------------------------------------------------|----|
| 464 gm. Monastral Green press cake (140 gm. pigment) | 40 |
| 109 gm. Resimene 888                                 |    |
| 54 gm. blown castor oil                              | 45 |
| 54 gm. butyl Cellosolve                              |    |
| Flush and remove 315 gm. water                       | 50 |
| 68 gm. ethyl cellulose 10 cp.                        |    |
| Mix until dissolved                                  | 55 |
| 300 gm. water                                        |    |
| Wash and remove 300 gm. water                        | 60 |
| 300 gm. water                                        |    |
| Wash and remove 300 gm. water                        | 65 |
| 300 gm. water                                        |    |
| Wash and remove 300 gm. water                        | 70 |
| 50 gm. Pflaumer's ester P-153-S                      |    |
| 50 gm. Triton X-100                                  | 75 |
| 25 gm. ammonia (27% NH <sub>3</sub> )                |    |
| 441 gm. water                                        |    |
| 2,215 gm.                                            |    |

Uses a natural oil-type plasticizer.

## EXAMPLE XII

The materials employed, with a brief indication as to the steps, are as follows:

|                                                                   |    |
|-------------------------------------------------------------------|----|
| 109 gm. Resimene 888                                              | 55 |
| 54 gm. dibutyl phthalate                                          |    |
| 54 gm. butyl Cellosolve                                           | 60 |
| 140 gm. Vulcan Red BA (General Dyestuff Corp. Pat. No. 1,977,936) |    |
| Mix and grind on roller mill, transfer to mixer. Add:             | 65 |
| 68 gm. ethyl cellulose 10 cp.                                     |    |
| 50 gm. Triton X-100                                               | 70 |
| 20 gm. ammonia (27% NH <sub>3</sub> )                             |    |
| 505 gm. water                                                     |    |
| 1,000 gm.                                                         |    |

In this example a dry pigment was ground into the resin vehicle with a sufficient loss of volatile, water-soluble, butyl Cellosolve so as not to interfere with the emulsification.

In the above examples there have been made padding colors for dyeing textile fabrics by flushing or grinding water-insoluble pigments in a resin solution containing:

Alkylated melamine formaldehyde resin

A non-volatile plasticizer

A water-soluble volatile organic solvent, capable of dissolving the resin and ethyl cellulose, and largely removed during the compounding steps. This solution may or may not include a cellulose ether.

After flushing or grinding, the ethyl cellulose, not included in the original solution is dissolved. If the color has been flushed from a water dispersion or presscake, a washing operation to remove most of the water-soluble volatile organic solvent is performed. In the cases where dry pigment is ground into the resin solution, this removal of volatile solvent is accomplished by evaporation. After the incorporation of a suitable amount of emulsifier, this mass is then capable of being dispersed in water by the slow addition of water.

The resulting product is a resin bound pigment dispersed in water containing no water-insoluble volatile solvents, and only very small quantities of water-soluble solvents. The dispersion in water is so fine that penetration into the threads and around the fibres of a fabric is

system for the purpose of facilitating the formation of a stable emulsion of the principal ingredients.

With respect to the pigments employed in these compositions, it is desirable that they be inert with respect to the balance of the compositions, insoluble in both the resin and the aqueous phases and be fast to light. Resistance to dry cleaning fluids is also a desirable characteristic of these compositions, but for temporary displays, for example, the desirable characteristics of light fastness, washability, etc. are not essential. In the dyeing of textiles which are to have a more permanent use, the pigments should be non-bleeding, light fast, and unaffected by cleaning solutions and soaps. Pigments suitable for use in this connection are well known and while an essential component of the compositions of this invention, they do not have a distinguishing class of characteristics other than insolubility in both of the phases of the completed emulsion.

For what may be a clearer presentation of the compositions of this invention, in the table below there have been tabulated the compositions of the preceding 12 examples in terms of parts per 1,000 parts of concentrated composition.

Table I

| Example No.             | I     | II    | III   | IV    | V     | VI    | VII   | VIII  | IX    | X     | XI    | XII   |
|-------------------------|-------|-------|-------|-------|-------|-------|-------|-------|-------|-------|-------|-------|
| Melamine-aldehyde resin | 136   | 86    | 83    | 112   | 109   | 89    | 100   | 109   | 109   | 109   | 109   | 109   |
| Cellulose ether         | 68    | 54    | 52    | 70    | 68    | 56    | 48    | 68    | 68    | 68    | 68    | 68    |
| Plasticizer             | 136   | 86    | 83    | 112   | 54    | 44    | 54    | 54    | 54    | 54    | 54    | 54    |
| Pigment                 | 68    | 107   | 104   | 140   | 136   | 112   | 140   | 140   | 140   | 140   | 140   | 140   |
| Deflocculating agent    | 8     | 27    | 9     | 12    | 34    | 28    | —     | 54    | 47    | 70    | 54    | 54    |
| Water-soluble solvent   | 16    | 30    | 41    | 46    | 49    | 86    | 104   | —     | —     | —     | 55    | 55    |
| Emulsifying agent       | 54    | 93    | 89    | 61    | 105   | 87    | 107   | 107   | 107   | 107   | 107   | 107   |
| Water                   | 514   | 517   | 539   | 447   | 446   | 498   | 438   | 468   | 475   | 452   | 468   | 520   |
| Total                   | 1,000 | 1,000 | 1,000 | 1,000 | 1,000 | 1,000 | 1,000 | 1,000 | 1,000 | 1,000 | 1,000 | 1,000 |

so complete that a uniform dyeing effect is obtained when the textile is padded, dried to remove the water, and cured.

Furthermore, superior fastness properties are obtained, when the fabric is dried and the resin polymerized, because the distribution of the resin and pigment is so even and the penetration so complete.

Unlike systems where water dispersions of pigments are added to resin latices, this system has superior fastness properties because the pigment is dispersed in the resin phase and is deposited with it on the fabric, and not left to chance that a particle of pigment will find a particle of binder.

The plasticizers suitable for this process include any that are compatible with both ethyl cellulose and butylated melamine formaldehyde.

The water-soluble volatile solvents useful in rendering the melamine aldehyde resin more workable include methyl alcohol, ethyl alcohol, propyl alcohol, isopropyl alcohol, acetone, diacetone alcohol, methyl Cellosolve (monomethyl ether of ethylene glycol), Cellosolve (monoethyl ether of ethylene glycol), isopropyl Cellosolve (monoisopropyl ether of ethylene glycol), butyl Cellosolve (monobutyl ether of ethylene glycol), methyl acetate.

The Blancol solution used in the foregoing examples is a deflocculating agent for the presscake, and any other suitable deflocculating agent such as the sodium lignosulfonates may also be employed for this purpose. It should be noted that in certain instances such deflocculating agents are not required. The fatty acid, hydroxyl amine and ammonia appearing in certain of the foregoing examples is an emulsification agent

The foregoing table illustrates preferred concentrations of the various components in the preferred compositions illustrated by Examples I through XII. Such ingredients may have the following preferred ranges of concentration for most satisfactory results:

Melamine-aldehyde resin—from about 8 to about 11 parts/100  
 Cellulose ether—from about 4.5 to about 7 parts/100  
 Plasticizer—from about 4 to about 17 parts/100  
 Pigment—from about 7 to about 14 parts/100  
 Deflocculating agent—from 0 to about 3.5 parts/100  
 Water-soluble solvent—from about .5 to about 10.4 parts/100  
 Emulsifying agent—from about 5 to about 11 parts/100  
 Water—from about 43 to about 54 parts/100

These are to be construed as preferred ranges from which variations may be made without departing from the spirit of this invention. With respect to the water-soluble solvent, however, it should be pointed out that these figures are somewhat misleading and, in all probability, somewhat high in value since during many of these operations, these low boiling water-soluble organic solvents are lost by evaporation to a much larger degree than is represented in the table above. Analysis has shown that in most cases the water-soluble solvent content in the concentrated materials rarely exceeds 5% by weight. The figures in the foregoing table are calculated by weight balance from the preceding specific examples, in which calculations no allowance has been made for evaporation of the solvent during the formu-

lating process. As indicated above, however, final analysis of the concentrated compositions has shown that in general, the amount of such solvent is less than 5% by weight of the entire composition.

It should also be borne in mind that these concentrates are used in making a pad dyeing bath in which baths the concentration of the concentrates never exceeds about 10% by weight, and generally is used at a concentration of about 2.5%. Smaller amounts of the concentrate may be used. Since no more than about 10% of this pigmented emulsion would be included in a dye bath for application onto textile materials, the amount of volatile solvents in the dye bath would be 1% or less and for the purposes of this invention a maximum amount of 1% of such water-soluble organic solvents is to be construed as substantially no solvent appearing in the final pad dyeing bath. Water may be added to the concentrates of this invention to effect the desired reduction to pad dyeing bath concentration, the amount of water so added being generally in the range of from about 90 to about 99 parts per 100 parts of finished pad dyeing bath, and preferably from about 95 to about 97.5 parts of water per 100 parts of bath, the balance being a concentrate such as exemplified above.

Other modes of applying the principle of this invention may be employed instead of those specifically set forth above, changes being made as regards the details herein disclosed, provided the elements set forth in any of the following claims, or the equivalent of such be employed.

I, therefore, particularly point out and distinctly claim as my invention:

1. A resin-in-water emulsion suitable for use in pad dyeing baths in which the resinous binder comprises a water-insoluble cellulose ether, a water-insoluble alkylated melamine-aldehyde resin and a non-volatile plasticizer, said resinous binder having dispersed therein an insoluble pigment, and in which emulsion the aqueous phase comprises water, said emulsion being free of water-insoluble organic solvents and containing less than 5% by weight of a water-soluble organic solvent.

2. A pad dyeing composition of the resin-in-water emulsion type in which the resinous binder comprises a water-insoluble cellulose ether, a water-insoluble alkylated melamine-formaldehyde resin and a non-volatile plasticizer, said resinous binder having dispersed therein an insoluble pigment, and in which the aqueous phase comprises water, said composition containing no water-insoluble volatile organic solvent and less than 1% by weight of a water-soluble volatile organic solvent.

3. A resin-in-water emulsion suitable for use in pad dyeing baths in which the resinous binder comprises a water-insoluble cellulose ether, a water-insoluble alcohol modified methylol-melamine and a non-volatile plasticizer, said resinous binder having dispersed therein an insoluble pigment, and in which emulsion the aqueous phase comprises water, said emulsion being free of water-insoluble organic solvents and containing less than 5% by weight of a water-soluble organic solvent.

4. A composition in accordance with claim 1 in which the alkylated melamine-aldehyde resin is a melamine-formaldehyde resin modified with an aliphatic alcohol containing from 3 to 12 carbon

5. A composition in accordance with claim 1 in which the alkylated melamine-aldehyde resin is a

melamine-formaldehyde resin modified with butyl alcohol.

6. A composition in accordance with claim 1 in which the cellulose ether is an aliphatic cellulose ether.

7. A composition in accordance with claim 1 in which the cellulose ether is an alkyl cellulose ether.

8. A composition in accordance with claim 1 in which the cellulose ether is ethyl cellulose having an ethoxy content within the range of from about 40% to about 50%.

9. A composition in accordance with claim 1 in which the amount of cellulose ether by weight is no more than the amount of alkylated melamine-aldehyde resin by weight.

10. A resin-in-water emulsion suitable for use in pad dyeing baths in which the resinous binder comprises a water-insoluble ethyl cellulose having an ethoxy content within the range of from about 40% to about 50%, a water-insoluble butylated melamine-formaldehyde resin and a non-volatile plasticizer, said resinous binder having dispersed therein an insoluble pigment, and in

15 which emulsion the aqueous phase comprises water, said emulsion being free of water-insoluble organic solvents and containing less than 5% by weight of a water-soluble organic solvent, and in which composition, the ratio of ethyl cellulose to butylated melamine-formaldehyde resin is no more than 1 part of ethyl cellulose to 1 part of resin by weight.

11. The method of pad dyeing to produce a solid color effect which comprises subjecting textile materials having discrete fibers to a resin-in-water emulsion in which the resinous binder comprises a water-insoluble cellulose ether, a water-insoluble alkylated melamine-aldehyde resin and a non-volatile plasticizer, said resinous binder having dispersed therein an insoluble pigment, and in which emulsion, the aqueous phase comprises water, said emulsion being free of water-insoluble organic solvents and containing less than 1% by weight of a water-soluble organic solvent, and then drying the material to remove the water.

12. The product produced by the method of claim 11.

13. A pad dyeing bath for textiles comprising a water reduction of the following composition, the amount of water used for said reduction being from about 90 to about 99 parts per 100 parts of pad dyeing bath:

55 Melamine-aldehyde resin—from about 8 to about 11 parts per 100 parts concentrate;  
Water-insoluble cellulose-ether—from about 4.5 to about 7 parts per 100 parts concentrate;  
Non-volatile plasticizer—from about 4 to about 17 parts per 100 parts concentrate;  
Deflocculating agent—up to about 3.5 parts per 100 parts concentrate;  
Organic water-soluble solvent—from about 0.5 to about 10.4 parts per 100 parts concentrate;  
Emulsifying agent—from about 5 to about 11 parts per 100 parts concentrate;  
Water—from about 43 to about 54 parts per 100 parts concentrate.

14. The method of pad dyeing to produce a solid color effect which comprises subjecting textile materials having discrete fibers to a resin-in-water emulsion in which the resinous binder comprises a water-insoluble ethyl cellulose having an ethoxy content within the range of from about 40% to about 50%, a water-insoluble butylated

13

melamine formaldehyde resin and a non-volatile plasticizer, said resinous binder having dispersed therein an insoluble pigment, and in which the aqueous phase comprises water, said emulsion being free of water-insoluble organic solvents and containing less than 1% by weight of a water-soluble organic solvent, and in which composition the ratio of ethyl cellulose to butylated melamine formaldehyde resin is no more than 1 part of ethyl cellulose to 1 part of resin by weight, and then drying the material to remove the water.

14

15. The product produced by the method of claim 14.

JOSEPH M. KUHN.

5 REFERENCES CITED

The following references are of record in the file of this patent:

UNITED STATES PATENTS

10 Number Name Date  
2,527,530 Cassel ----- Oct. 31, 1950